

## UNITED STATES PATENT OFFICE

2,144,249

CATHODE FOR ELECTRON DISCHARGE  
DEVICES

Victor O. Allen, Madison, N. J., assignor, by mesne assignments, to Radio Corporation of America, New York, N. Y., a corporation of Delaware

No Drawing. Application February 23, 1935,  
Serial No. 7,853

7 Claims. (Cl. 250—27.5)

My invention relates to electron discharge devices, more particularly to improvements in thermionic electron emitting cathodes for such devices.

5 The present application relates to modifications of the invention described and claimed in co-pending United States patent application, Serial No. 43,714, filed October 5, 1935, by Victor O. Allen and Joseph Johnson as joint inventors, 10 and assigned to the same assignee as the present invention.

In conventional electron discharge devices with the filament type of thermionic cathode commercial use has been made of pure tungsten filaments, 15 activated thoriated tungsten filaments, and oxide coated nickel filaments. The pure tungsten filament cathode is a very stable emitter and is efficient but must be operated at very high temperatures to obtain ample emission. The activated thoriated tungsten cathode, such as described in U. S. patent to Langmuir 1,244,216, 20 may be operated at lower temperatures than a pure tungsten filament and is more efficient, but is easily poisoned by oxygen and other gases 25 which adversely affect the emission, is not very stable when operated at high voltages, and requires special processing and seasoning. It has also been found that when operated at ultra-high frequencies, for example above 15 or 16 30 megacycles, that emission becomes erratic and that there is sometimes a total loss of emission. In addition, the activated thoriated filament is apt to be brittle, and if operated at too high a temperature quickly deactivates and loses its 35 ability to emit a sufficient number of electrons to be useful. The oxide coated nickel cathode operates at a much lower temperature than either kind of tungsten cathode and is efficient, but cannot be satisfactorily operated in tubes in which 40 very high plate voltages, such as 1000 volts, are used, and requires considerable processing and seasoning.

Thoriated molybdenum has also been thoroughly investigated as a filament cathode emitter, 45 but has proved to be rather unstable, quite sensitive to poisoning by gas within the tube, and must be operated at fairly high temperatures, between 1400° and 1600° C. to provide satisfactory emission. For these and other reasons thoriated 50 molybdenum has not come into commercial use as a cathode filament material.

In the conventional high vacuum or gas tube operating at high voltages, only filamentary type cathodes have heretofore been used because the 55 oxide coatings of the indirectly heated cathodes

quickly disintegrate at high voltages, and without these coatings no material was available which had sufficient emission unless raised to very high temperatures which cannot be practically generated with the conventional indirectly heated cathode construction.

An object of my invention is to provide a ductile thermionic cathode which is a stable, efficient and long lived emitter, at desirable operating temperatures. A further object is to provide an 10 efficient thermionic cathode which can be satisfactorily used at high frequencies and high voltages and requires little seasoning or processing. Another object of my invention is to provide an 15 indirectly heated cathode for high voltage gas or vacuum tubes.

In accordance with my invention I use a refractory metal having a high melting point, preferably 2400° C. or higher combined with thoria and chromium or their equivalents. Of these 20 refractory metals I prefer to use tungsten, molybdenum or tantalum. The thoria may be incorporated in the tungsten metal to form a base, and the chromium plated on the thoriated tungsten base, or the pure tungsten, molybdenum 25 or tantalum base may be chromium plated and the thoria applied as a coating on the plated base.

The thoriated tungsten base may be prepared as a ductile metal in accordance with U. S. Patent 30 1,082,933 to W. D. Coolidge, or by squirting the finely divided material admixed with a binder. For example, if tungsten is used I may add powdered nitrate of thoria to the powdered oxide of tungsten before the reduction of the oxide of 35 tungsten, or I may add thoria to the oxide of tungsten after reduction but before consolidation of the metal powder by sintering and mechanical working to the solid state as described in the said Coolidge patent. The amount of thoria may 40 vary from about  $\frac{1}{2}$  of 1% by weight of the metal to about 3% of the metal. Tungsten containing more than 2% or 3% of thoria is extremely brittle and hard to work, but in general 45 I have found it desirable for best results to add as much thoria as may be tolerated in the refractory metal without interfering with the subsequent swaging and drawing of the metal. This has been found in practice to be up to 1½% for tungsten. A filament of this thoriated metal 50 may be used. In general the larger the percentages of thoria the better the emitter. While thoria is preferred, equivalents of thoria, for example one of the group of metals consisting of zirconium, uranium, cerium, titanium, vanadium, 55

yttrium and lanthanum may be used with tungsten to form a base and the base then chromium plated in a conventional chromium plating bath, the essential constituents of which are chromic acid and a sulphate. One example of a satisfactory bath is 33 oz. chromic acid, containing at least 95% chromium oxide ( $\text{CrO}_3$ ) and not more than 0.2%  $\text{SO}_4$ , and .45 gram chemically pure sulphuric acid ( $\text{H}_2\text{SO}_4$ ) in a gallon of water. The limits of thickness of the chromium plating may be wide, although a very thin plating appears to be entirely satisfactory. While the current density for plating the chromium on the thoriated metal base may vary between wide limits, for example, from a few hundredths of an ampere to over 1 ampere per square centimeter, for best results a current density of about 1 ampere per square centimeter for a period of one minute seems to produce the most satisfactory results. The resulting chromium plated thoriated wire may be used for a thermionic electron emitting cathode without further treatment, but for best results in the case of the thoriated tungsten base I prefer to flash the plated filament in vacuum at over voltage; for example, to heat the filament to a temperature of approximately  $2600^{\circ}$  K. for about thirty seconds, and thereby facilitate the activation of the filament. It is also desirable, though not necessary, to insure stability of emission to season the filament by operating the electron discharge device containing the filament with normal voltages applied for approximately fifteen minutes in an oscillating circuit.

A cathode made in accordance with my invention has a normal operating temperature several hundred degrees K. below the normal operating temperature of the conventional activated thoriated tungsten cathode, and in the conventional type of tube operated at the customary plate voltage the same plate current can be obtained from my improved cathode at its normal operating temperature with only about one-half the energy per unit area that must be used to obtain the same plate current from the conventional activated thoriated tungsten cathode at its normal operating temperature.

While I do not wish to be limited to any particular theory it is believed that the chromium acts as a catalyst to facilitate the rapid diffusion of the electron emitting metal, such as thorium, to the surface of the filament for producing copious emission.

A pure tungsten, molybdenum, or tantalum filament may be chromium plated as above described and then brushed with thoria powder suspended in acetone and of a particle size which will pass thru a 200 mesh screen or smaller. This will also provide a very efficient emitter. The thickness of the coating should come within the limits described above. Treatment to insure stability of emission as described above is desirable but not necessary.

When the cathodes are to be used in low voltage tubes, for example under 1000 volts, to increase the electron emissivity any of the cathodes above described may be coated with the usual electron emitting coating of alkaline earth metal oxides, such as barium oxide and strontium oxide, which may be applied in a conventional manner by applying barium and strontium carbonates and converting them into the oxides.

A cathode made in accordance with my inven-

tion is a very efficient emitter. It will operate at a comparatively low temperature ( $1200^{\circ}$  K.) and very high voltages can be used on the plate of a tube using my cathode up to approximately 3000 volts without the cathode suffering any ill effects due to ion bombardment. These last two characteristics make my invention particularly suitable for indirectly heated cathodes in high voltage gas or vacuum tubes.

Cathodes made according to my invention are very satisfactory in tubes used for generating very high frequencies at high voltages and while seasoning improves the initial stability and operating characteristics it is not essential in order to provide a cathode which is a good emitter and operates satisfactorily. The resulting cathode is a very stable emitter and is not easily poisoned by gas. The cathode readily recovers its emitting characteristics even if accidentally operated temporarily at too high temperatures. High voltage ionization will not destroy the tube due to ion bombardment, and the cathode will recover its emission if temporarily impaired by being subjected to high voltages.

While I have indicated the preferred embodiment of my invention of which I am now aware and have also indicated only certain specific application for which my invention may be employed, it will be apparent that my invention is by no means limited to the exact forms illustrated or the use indicated, but that many variations may be made in the particular structure used and the purpose for which it is employed without departing from the scope of my invention as set forth in the appended claims. 35

What I claim as new is:

1. A thermionic cathode adapted for use as an electron emitter in electron discharge devices comprising a refractory metal body consisting predominantly of tungsten, and the remainder containing thoria and electrolytically applied chromium. 40

2. A thermionic cathode for use in an electron discharge device and consisting essentially of one of the group of metals tungsten and tantalum, in combination with electrolytically applied chromium and at least one of the group of substances consisting of thoria, zirconium, uranium, cerium, titanium, vanadium, yttrium and lanthanum. 45

3. A thermionic cathode for use in an electron discharge device and consisting essentially of tungsten and containing thoria and a coating of electrolytically applied chromium on the thoriated tungsten. 50

4. A thermionic cathode for use in an electron discharge device and consisting essentially of one of the group of metals, tantalum, tungsten or molybdenum and a coating of thoria and electrolytically applied chromium on said metal. 55

5. A thermionic cathode for use in an electron discharge device and comprising a metal of high melting point, a chromium plating on said metal and a coating of thoria on said chromium plating. 60

6. A thermionic cathode for use in an electron discharge device and comprising molybdenum, a chromium plating on said molybdenum and a coating of thoria on said chromium plating. 65

7. A thermionic cathode for use in an electron discharge device and comprising tungsten, a chromium plating on said tungsten and a coating of thoria on said chromium plating. 70

VICTOR O. ALLEN.

CERTIFICATE OF CORRECTION.

Patent No. 2,144,249.

January 17, 1939.

VICTOR O. ALLEN.

It is hereby certified that error appears in the printed specification of the above numbered patent requiring correction as follows: Page 2, second column, line 2, for "(1200° K.)" read (1200° C.); and that the said Letters Patent should be read with this correction therein that the same may conform to the record of the case in the Patent Office.

Signed and sealed this 18th day of July, A. D. 1939.

(Seal)

Henry Van Arsdale,  
Acting Commissioner of Patents.